

# United States Patent [19]

Hammond et al.

[11] 4,420,647

[45] Dec. 13, 1983

[54] SEMI-SYNTHETIC LUBRICATING OIL COMPOSITION

[75] Inventors: Kenneth G. Hammond, Poughkeepsie; Joseph C. Sendra, Fishkill, both of N.Y.; Lewis W. Watts, Jr., Austin, Tex.; Edward T. Marquis, Austin, Tex.; John M. Larkin, Austin, Tex.

[73] Assignee: Texaco Inc., White Plains, N.Y.

[21] Appl. No.: 371,859

[22] Filed: Apr. 26, 1982

[51] Int. Cl.<sup>3</sup> ..... C10M 1/18; C07C 1/16; C07C 3/18

[52] U.S. Cl. ..... 585/10; 585/12; 585/18; 585/255; 585/510; 585/525; 585/643

[58] Field of Search ..... 585/10, 12, 18, 255, 585/510, 512, 520, 526, 525, 532, 643, 648, 660, 664

[56] References Cited

U.S. PATENT DOCUMENTS

3,152,998 10/1964 Moss ..... 252/474  
3,780,128 12/1973 Shubkin ..... 585/12  
4,042,488 8/1977 Perciful ..... 585/648

4,045,508 8/1977 Cupple et al. ..... 585/517  
4,218,330 8/1980 Shubkin ..... 252/46.6  
4,300,006 11/1981 Nelson ..... 585/525

Primary Examiner—Jacqueline V. Howard  
Attorney, Agent, or Firm—Jack H. Park; Kenneth R. Priem; David L. Mossman

[57] ABSTRACT

A synthetic lubricating oil composition comprising a major portion of a synthetic lubricant component or a mixture of a synthetic lubricant component and a hydrocarbon mineral base oil and a minor portion of various additive components is described. The synthetic lubricant component is manufactured from internal olefins.

The process for making the synthetic lubricant component utilizes boron trifluoride catalysis with a promoter to produce oligomer mixtures that have surprisingly low viscosities at low temperatures and surprisingly high viscosity indexes as compared with the oligomers found in other methods. It is important that internal olefins be used predominantly to make the oligomers. Alpha olefins make up the balance of the olefins.

23 Claims, No Drawings

## SEMI-SYNTHETIC LUBRICATING OIL COMPOSITION

## CROSS-REFERENCE TO RELATED APPLICATIONS

This application is related to co-pending patent application Ser. No. 372,492, filed on Apr. 28, 1982, which is related to the manufacture of synthetic lubricant additives over boron trifluoride from mixtures of C<sub>9</sub>–C<sub>24</sub> olefins comprising greater than 99 weight percent of the mixture, with no limitation on the source of the internal olefins.

This application is also related to co-pending patent application Ser. No. 372,491, filed Apr. 28, 1982, which is related to the manufacture of synthetic lubricant additives over boron trifluoride from mixtures of alpha and internal olefins where internal olefins are greater than 50 but less than 99 weight percent of the mixtures.

## BACKGROUND OF THE INVENTION

## 1. Field of the Invention

The invention relates to lubricating oil compositions, and more particularly relates to lubricating oil compositions incorporating oligomers made from predominantly internal olefins by means of a boron trifluoride catalyst.

## 2. Description of Related Methods

Friedel-Crafts catalysts have long been known to oligomerize olefins. For example, see U.S. Pat. No. 3,410,925 to Eby, et al. in which olefins are mixed with alkylatable aromatic hydrocarbons over a Friedel-Crafts catalyst to form an alkylation sludge which is then mixed with olefins having 3 to 18 carbon atoms which are also passed over the catalyst to produce olefin dimers. U.S. Pat. No. 3,652,706 to Saines, et al. describes the polymerization of olefins having 2 to 20 carbon atoms over a Friedel-Crafts metal halide catalyst plus a hydrogen form of mordenite to produce compounds having a molecular weight between 700 and 2,500. Production of a gasoline fuel composition is described in U.S. Pat. No. 3,749,560 to Perilstein which occurs by reacting a mixture of mono olefins (greater than 50 weight percent alpha olefins) over a Friedel-Crafts catalyst heated to a temperature around 145° C. to produce oligomers having molecular weights between 350 to 1,500. Also, U.S. Pat. No. 3,149,178 to Hamilton, et al. reveals an improved method for making polymerized olefin synthetic lubricants via a particular distillation technique of oligomers made from alpha mono olefins using a Friedel-Crafts catalyst. Alpha olefins having six to twelve carbon atoms may be dimerized in the presence of a Friedel-Crafts catalyst according to the method described in U.S. Pat. No. 4,172,855 to Shubkin, et al.

It is also known that the term "Friedel-Crafts catalysts" includes boron trifluoride among other metal halide-type Lewis catalysts, see *Kirk-Othmer Encyclopedia of Chemical Technology*, Third Edition, Vol. 11, pg. 292. Boron trifluoride has also been known to polymerize olefins, as seen in F. Albert Cotton, et al., *Advanced Inorganic Chemistry: A Comprehensive Text*, Interscience Publishers, 1962, p. 191.

A number of U.S. patents have also used BF<sub>3</sub> to oligomerize olefins. Close study will reveal that alpha olefins are considered the only useful form. For example, U.S. Pat. No. 2,780,664 to Serniuk describes the reaction of conjugated dienes with mono alpha and

internal olefins over BF<sub>3</sub> promoted by an ether mixed with a halo alkane diluent at a temperature from –30° to 100° C. to produce oligomers suitable for drying oils. Alpha olefins having from 5 to 20 carbon atoms are oligomerized using BF<sub>3</sub> plus an alcohol or water promoter as described in U.S. Pat. No. 3,382,291 to Brennan. In this patent, BF<sub>3</sub> and a mixture of BF<sub>3</sub> plus the promoter complex are introduced in two separate streams. Another U.S. patent by Brennan, U.S. Pat. No. 3,742,082, concerns the dimerization of alpha olefins via BF<sub>3</sub> which is promoted with phosphoric acid or water at a temperature from 100° to 150° C. U.S. Pat. No. 3,763,244 to Shubkin, which describes the oligomerization of n-alpha olefins having 6 to 16 carbon atoms over BF<sub>3</sub> promoted with water, at a temperature between 10° and 60° C. where it is preferred that BF<sub>3</sub> is added continuously.

Yet another U.S. patent to Brennan, U.S. Pat. No. 3,769,363, describes the oligomerization of olefins having 6 to 12 carbon atoms using BF<sub>3</sub> with a carboxylic acid promoter having at least 3 carbon atoms at a temperature between 0° and 20° C. to produce olefins heavy in trimer form. U.S. Pat. No. 3,780,128 also to Shubkin relates to the oligomerization of alpha olefins having 6 to 16 carbon atoms in which BF<sub>3</sub> is employed in a molar excess of alcohol. U.S. Pat. No. 3,876,720 to Heilman, et al. describes a two-step procedure by which alpha olefins having 8 to 12 carbon atoms are converted to vinylidene olefins which are then reacted over a 1:1 molar complex of BF<sub>3</sub> and alcohol to produce oligomerized vinylidene olefins. A method for oligomerizing both short and long chain alpha olefins having from 14 to 20 carbon atoms simultaneously over BF<sub>3</sub> with an alcohol or water promoter at 0° to 60° C. with a monomer recycle is described in U.S. Pat. No. 4,225,739 to Nipe, et al. There is also U.S. Pat. No. 4,263,465 to Sheng, et al. which describes a two-step process for reacting one-butene with a higher alpha olefin over BF<sub>3</sub> in the presence of a proton donor at a temperature from –30° to 50° C. to produce an oligomer having 8 to 18 carbon atoms. The intermediate oligomer is reacted with other higher alpha mono olefins over the same catalyst system from –30° to 60° C. to produce oligomers having 20 to 40 carbon atoms. For more information on BF<sub>3</sub>-catalyzed oligomerization of alpha olefins, see Brennan, "Wide-Temperature Range Synthetic Hydrocarbon Fluids," Ind. Eng. Chem. Prod. Res. Dev. 1980, Vol. 19, pp 2–6 and Shubkin, et al., "Olefin Oligomer Synthetic Lubricants: Structure and Mechanism of Formation," Ind. Eng. Chem. Prod. Res. Dev. 1980, Vol. 19, pp 15–19.

Two patents have been located which involve the reaction of internal olefins over Friedel-Crafts catalysts. U.S. Pat. No. 4,167,534 to Petrillo, et al. describes olefins which are both alpha and internal having from 10 to 15 carbon atoms which are reacted over Friedel-Crafts catalysts between 20° and 200° C. to produce oligomers. The catalysts used in the examples of this patent are only AlCl<sub>3</sub> and NaAlCl<sub>4</sub>. The internal olefins are also those that are statistically distributed. Also, the oligomers found useful therein seem to be the hydrogenated bottoms product after the unreacted olefins are removed, without further distillation. U.S. Pat. No. 4,218,330 to Shubkin describes hydrogenated dimers from alpha olefins having from 12 to 18 carbon atoms, especially 1-tetradecene, made using a Friedel-Crafts catalyst, which includes therein boron trifluoride with a

promoter. Shubkin's method uses predominantly alpha olefins, although the specification mentions that "fairly large amounts of internal olefins can be tolerated without adversely affecting the physical properties of the oligomer." This last remark from Shubkin reveals the general feeling of those working in the field that internal olefins do not produce oligomers with good properties for synthetic lubricants. For example, in U.S. Pat. No. 3,952,071 to Isa, et al., it is revealed that olefins may be oligomerized in the presence of a mixture of a polyhydric alcohol derivative and an aluminum halide. Isa, et al. mention that the olefin could be internal or alpha although alpha olefins are the only ones used in the examples therein. U.S. Pat. No. 3,947,509, also to Isa, et al., also claims that internal olefins may be used over a ketone and ester ether or alcohol promoted aluminum chloride catalyst although only alpha olefins are used in the examples.

U.S. Pat. No. 4,300,006 was issued on Nov. 10, 1981. It describes a process for producing a hydrocarbon oil by contacting a mixture of alpha and at least 50 weight percent internal olefins with a boron trifluoride dimerization catalyst. However, the productivity of useful products from the process revealed in U.S. Pat. No. 4,300,006 is quite low. For example, an alkane diluent is found to be necessary in the process described therein which, in addition to distilling out the lights and the heavies to obtain the lube oil, results in little useful product. Further, this method requires a much longer reaction time and a higher catalyst concentration than desired. It would be beneficial if a method for producing synthetic lubricant components could be devised which would overcome the aforementioned disadvantages.

In the field of synthetic lubricants, it is a continual problem to produce synthetic lubricant components having viscosities and other properties which permit them to be excellent motor oils.

#### SUMMARY OF THE INVENTION

The invention relates to a lubricating oil composition comprising a major portion of a synthetic lubricant component or a mixture of synthetic lubricant component and a lubricating hydrocarbon mineral base oil, the synthetic lubricant component being made by contacting a mixture of olefins having between 9 and 24 carbon atoms, inclusive, and having greater than 50 weight percent internal olefins, the balance being alpha olefins, with a catalyst comprising boron trifluoride together with a promoter at a reaction temperature sufficient to effect oligomerization of said olefins, then hydrogenating the oligomerized olefins to make the synthetic lubricant component, and minor portions of additive components.

#### DESCRIPTION OF THE PREFERRED EMBODIMENTS

It has been surprisingly discovered that oligomers which have an unusual blend of properties may be made by reacting predominantly internal mono olefins with boron trifluoride and a promoter. These oligomers are particularly useful in making excellent synthetic and semi-synthetic lubricating fluids. It must be stressed that this discovery has not been found by any of the other researchers in the field. It is also important to note that predominantly internal olefins are employed in the method of this invention.

Generally, the olefins should have between 9 and 24 carbon atoms, inclusive. It is preferred that only linear olefins be used. The internal olefins used herein have the double bond randomly distributed across the molecule. 5 In this context, the term "randomly distributed" means that the double bond in the internal olefin is not predominantly in any one location. For example, an olefin mixture being comprised of a majority of alpha olefins would be outside the scope of this definition since the 10 double bond would be located predominantly between the first and second carbon atoms of the molecules. Likewise, since the internal olefins used for oligomerization in the method of U.S. Pat. No. 4,300,006 are made by disproportionation of alpha olefins, the double 15 bond is located predominantly at or near the center of the molecule, and such olefin feedstocks also fall outside the definition of having a "random distribution" of the double bond. A random distribution includes the distribution one would obtain upon the dehydrogenation of 20 paraffins. One would expect a small amount of alpha olefin to result from such a distribution. However, it would be expected that the alpha olefin proportion would be only about 0.1 weight percent, with a maximum value being about 1.0 weight percent. Alpha olefins 25 may be added to the internal olefins as long as the internal olefins comprise more than half of the olefins present. As will be shown, the invention works well even if the olefins used for oligomerization to the synlube component consist essentially only of internal olefins.

The internal olefins may be generally expressed as 30 compounds having the formula  $RCH=CHR'$  where R and R' are the same or different alkyl radicals of one to twenty-one carbon atoms. However, the total number 35 of carbon atoms should not exceed twenty four and should not be less than nine. The internal olefin mixtures are potentially more available than the pure cut alpha olefins and are potentially as cheap or cheaper than the corresponding pure cut alphas. It will be shown that the 40 method of this invention affords higher quality products and higher conversions than those obtained with  $AlCl_3$  and  $AlCl_4Na$  catalysts.

By careful selection of the molecular weight of the 45 feed olefins and the reaction conditions, it was found that a synthetic lubricant base oil with a specific viscosity can be made by the method of this invention which has superior properties over those made by other methods. For example, it has been found that a base oil having a 210° F. viscosity of about 4 centistokes with excellent properties can be made with internal olefins having 50 13 or 14 carbon atoms. A "four centistoke fluid" is a designation given to fluids used in lubricating oil compositions which generally have 210° F. viscosities of about 4 centistokes.

55 Kinematic viscosities at two standard temperatures are given in centistokes. The viscosity index (VI) is the change in viscosity with temperature such that the higher the number, the lower is the change in viscosity with temperature. Conversely, a low VI signifies a large change in viscosity with temperature. Pour point is a measure of the lowest temperature, in degrees Fahrenheit, at which the sample will begin to pour. Below that temperature the composition may generally be regarded as a solid. The thermogravimetric analysis (TGA) is a 60 measure of volatility via measuring the weight percent of sample remaining at 233° C. as the temperature is raised in a slow, uniform manner, usually 10° C. per minute. An oligomer product should have a TGA anal-

ysis with at least 80% of the sample remaining at 233° C. in order to have sufficiently low volatility to be useful as a base stock for lube oil formulation.

Preferably, a "4 centistoke fluid" (measured at 210° F.) should have a viscosity between 25 and 40 centistokes at 25° C., a viscosity between 3.5 and 5.0 centistokes at 210° F., a viscosity index of greater than 100, a pour point of less than -50° F. and a thermogravimetric analysis percent remaining at 233° C. value of greater than 80 weight percent. It is especially preferred that 4 centistoke fluids have a viscosity of between 25 and 34 centistokes at 25° C., a viscosity between 3.5 and 4.5 cSt at 210° F., a minimum viscosity index of 110, a maximum pour point of less than -50° F. and a thermogravimetric analysis value of 86 weight percent, mini-

5

discharged, separated from the heavy catalytic layer, washed with caustic solution and then distilled.

Example 5 begins by adding the olefin feed at room temperature with 1% AlCl<sub>3</sub> in only one portion. The temperature is allowed to rise on its own for 120 minutes. The product is then discharged, separated from the heavy catalytic layer, washed with caustic solution and distilled.

The feed in Example 7 of U.S. Pat. No. 4,167,534 is added at 130° C. with 5% NaAlCl<sub>4</sub> over 90 minutes. The reaction mass is then maintained at 130° C. for 60 minutes further. The product is then discharged, separated from the heavy catalytic layer, washed with caustic solution and distilled. The results of the comparative examples are shown in Table I.

TABLE I

## COMPARATIVE EXAMPLES

| Example | Reaction Conditions      |                     | Temperature, °C. | Method of U.S. Pat. No. 4,167,534 | Conversion Basis LC | % Bottoms Basis Olefin Charged | Properties of Hydrogenated Stripped Oligomer |        | TGA: % Sample Remaining at 233° C. |
|---------|--------------------------|---------------------|------------------|-----------------------------------|---------------------|--------------------------------|----------------------------------------------|--------|------------------------------------|
|         | Feed                     | Catalyst            |                  |                                   |                     |                                | 210° F.                                      | 25° C. |                                    |
| 1       | C <sub>13</sub> -14 int. | AlCl <sub>3</sub>   | 80               | Ex. 1                             | 32.5                | 21.6                           | 5.69                                         | 56.00  | 127.4 -50 91.8                     |
| 2       | C <sub>13</sub> -14 int. | AlCl <sub>3</sub> * | 80               | Ex. 1                             | 42.2                | 29.2                           | 5.85                                         | 60.96  | 121.4 <-50 91.3                    |
| 3       | C <sub>11</sub> -14 int. | AlCl <sub>3</sub>   | 80               | Ex. 1                             | —                   | 21.0                           | 6.79                                         | 80.39  | 116.9 <-50 88.5                    |
| 4       | C <sub>14</sub> alpha    | AlCl <sub>3</sub>   | 80               | Ex. 1                             | 85.9                | 80.2                           | 22.07                                        | 341.83 | 129.9 +20 98.2                     |
| 5       | C <sub>13</sub> -14 int. | AlCl <sub>3</sub>   | R.T.**           | Ex. 5                             | 24.8                | 16.8                           | 6.40                                         | 68.90  | 124.4 -50 92.2                     |
| 6       | C <sub>13</sub> -14 int. | AlCl <sub>3</sub> * | R.T.             | Ex. 5                             | 45.6                | 27.4                           | 6.43                                         | 71.75  | 122.1 <-50 91.4                    |
| 7       | C <sub>11</sub> -14 int. | AlCl <sub>3</sub>   | R.T.             | Ex. 5                             | 36.8                | 23.2                           | 7.12                                         | 86.72  | 116.5 <-50 89.5                    |
| 8       | C <sub>14</sub> alpha    | AlCl <sub>3</sub>   | R.T.             | Ex. 5                             | 93.9                | 87.6                           | 18.20                                        | 260.91 | 131.2 +10 98.3                     |
| 9       | C <sub>13</sub> -14 int. | NaAlCl <sub>4</sub> | 130              | Ex. 7                             | 42.0                | 30.3                           | 5.20                                         | 48.68  | 125.9 <-50 88.2                    |
| 10      | C <sub>11</sub> -14 int. | NaAlCl <sub>4</sub> | 130              | Ex. 7                             | 68.9                | 44.8                           | 6.96                                         | 87.04  | 114.0 -45 91.3                     |
| 11      | C <sub>14</sub> alpha    | NaAlCl <sub>4</sub> | 130              | Ex. 7                             | 100.0               | 87.1                           | 19.44                                        | 286.80 | 130.5 +15 96.0                     |

\*Twice as much AlCl<sub>3</sub> was used in these examples as described in the examples of U.S. Pat. No. 4,167,534

\*\*R.T. means room temperature

mum.

The catalyst of choice is boron trifluoride. A number of different kinds of promoters may be used, such as alcohols, carboxylic acids or water. It is especially preferred that 1-butanol be used as the promoter. The temperature range at which the oligomerization may be performed successfully is between 25° and 150° C., with an especially preferred range between 65° to 105° C. The pressure range of the reaction may run from atmospheric to 1000 psig. The oligomerization of the olefins may be conducted in a batch or continuous mode. First, the experimental methods will be described, and then the results will be tabulated.

## COMPARATIVE EXAMPLES

A number of comparative oligomerization examples were run using the procedures of U.S. Pat. No. 4,167,534, the disclosure of which is incorporated by reference herein. It is believed that this patent constitutes the closest prior art. The examples herein were patterned after Examples 1, 5 and 7 therein. These examples were chosen because they represented a wide variety of conditions, particularly temperature. The primary variable in the comparative examples is the olefin feed material, although sometimes twice the amount of AlCl<sub>3</sub> used in U.S. Pat. No. 4,167,534 is employed in an attempt to improve the conversion.

According to the disclosure in U.S. Pat. No. 4,167,534, Example 1 is begun by heating the feedstock to 80° C. The feedstock is then added over 15 minutes with 1% AlCl<sub>3</sub>. The temperature is then raised to 100° C. and maintained for 100 minutes. The product is then

With respect to the results outlined in Table I, the conversion is a weight percent of monomer oligomerized as determined by liquid chromatography. The weight percent of the bottoms as based on the olefin charged is given in the next column. While these two columns of data generally measure the same concept (notice the qualitative correlation), the applicants prefer to use "% conversion" while the inventors in U.S. Pat. No. 4,167,534 used the "% bottoms" method. Both are employed in the examples of Table I for comparative purposes.

## EXAMPLES ILLUSTRATING THE INVENTION

The following examples illustrate the method of the invention using BF<sub>3</sub> as the catalyst and only internal olefins as the olefin feed. Two examples are included using C<sub>14</sub> alpha olefin as the feedstock to show that an unsuitable oligomer mixture is produced. The oligomer from alpha olefins having 14 carbon atoms (1-tetradecene) was deficient in its low temperature properties for use in crankcase engine oils. Generally, pour point of a synthetic base oil candidate should at least be less than -50° F.

## EXAMPLE 12

A solution of 43.8 g C<sub>13</sub>-14-15 random internal linear olefins (53.4% C<sub>13</sub>, 45.0% C<sub>14</sub>, 0.5% C<sub>15</sub>, 1.1% paraffins) and 0.12 g 1-butanol in a nitrogen atmosphere was saturated with BF<sub>3</sub> at 25° C. by slow sparging for 25 minutes. Pot contents were maintained at 25°-27° C. by external cooling while 55.6 g of a solution of 55.0 g C<sub>13</sub>-14-15 olefins and 0.8 g 1-butanol was added over 1½ hours. Boron trifluoride saturation was maintained dur-

ing this addition and for 1 $\frac{1}{4}$  hours thereafter. Boron trifluoride introduction was stopped and the pot contents were heated to 86° C. over a 1 $\frac{1}{4}$  hour period, and maintained at 85°–86° C. for  $\frac{1}{2}$  hour. After cooling, 110 ml H<sub>2</sub>O was added; the contents were stirred rapidly for 20 minutes, and the top layer was removed. It was washed with 115 ml H<sub>2</sub>O and stripped on a rotary evaporator at 30 mm Hg to a maximum bath temperature of 95° C.; 96.9 g of a clear light yellow liquid remained (98.3% recovery). Analysis by gel permeation chromatography indicated 61.34% dimer, 25.13% trimer, and 12.95% monomer, the balance being higher oligomers.

#### EXAMPLE 13

The product of Example 12 (93.8 g) was hydrogenated over 9.60 g of a powdered Ni/Cu/Cr catalyst, which is described in U.S. Pat. No. 3,152,998, incorporated by reference herein. The conditions included a pressure of 1800 psig H<sub>2</sub> and a temperature of predominantly 208° C. (with temperature briefly reaching 316° C.).

Vacuum stripping was conducted at 0.9 mm Hg, with a maximum head temperature of 105° C. and a maximum pot temperature of 157° C., to remove 11.89 g of lighter components (>91% monomers). The hydrogenated bottoms product consisted (GPC analysis) of 26.7% trimer, >67.8% dimer, and >3.41% monomer. The kinematic viscosities at 25° C., 100° F., and 210° F. were 29.57, 18.26 and 3.89 centistokes, respectively. The pour point was measured to be less than –50° F. Thermogravimetric analysis indicated 81.3% of the sample remained at 233° C.

#### EXAMPLE 14

This is essentially the same procedure as Example 12 except BF<sub>3</sub> introduction was stopped when olefin/1-butanol introduction stopped. The heating period was for 2 hours at 90° C. GPC analysis indicated 19.8% trimer, 62.2% dimer and 17.94% monomer, the balance being higher oligomers.

#### Hydrogenation

In order to form materials which have adequate oxidative stability for lubricants, the oligomerized olefins are optionally hydrogenated either partially or totally. This hydrogenation is done by procedures known to those skilled in the art as exemplified by U.S. Pat. Nos. 4,045,508; 4,013,736; 3,997,622 and 3,997,621. A particularly preferred catalyst for this hydrogenation is a nickel-copper-chromia catalyst described in U.S. Pat. No. 3,152,998, incorporated by reference herein. As is well known, such hydrogenations may be performed in either batch or continuous modes.

When the instant inventive method was scaled up for a pilot plant run, it was discovered that the resulting oligomer mixture did not give the expected desirable properties seen in the lab scale experiments. In the pilot plant scale-up, stripping out the monomer was performed first and then hydrogenation was conducted over the nickel-copper-chromia catalyst described above. Monomer removal was performed before hydrogenation and recycled to the oligomerization step. However, during the pilot plant stripping step over 50% of the oligomer material came off overhead at temperatures starting at about 210° C. to about 282° C. at the finish in an attempt to obtain a material with a good TGA (volatility) value. Apparently, some of the unhydrogenated oligomer mixture was thermally unsta-

ble and portions of it were reverting to monomers or intermediates and distilling off as volatiles. It is, therefore, important that monomer removal be accomplished at as mild conditions as possible; that is, the reboiler or pot temperatures should preferably be kept at or under 180° C. when stripping out monomer.

While the methods of others in the field include a distillation step after hydrogenation procedure to obtain products of various 210° F. viscosities, it is much preferred in the method of the invention that no further distillation be conducted. In other words, the monomer-stripped, hydrogenated bottoms are the desired synthetic lubricant components. Thus the method of this invention does not require the customary distillation step, yet surprisingly produces a synthetic lubricant component that has excellent properties and performs in a superior fashion. However, it is also anticipated that one skilled in the art may find subsequent distillation useful in the practice of the method of this invention.

#### EXAMPLES 15–26

The following examples illustrating the method of the invention were conducted according to one of the following procedures.

##### Procedure A

Examples 15 through 18 used the following experimental procedure. To a 300 ml stainless steel clave (316 SS) was charged 158.6 g of olefin and 1.4 g of 1-butanol. The clave was sealed and heated to approximately 98° C. at which time BF<sub>3</sub> gas was introduced in amounts ranging from 3.1 to 4.4 g (average 3.8 g BF<sub>3</sub> per run). The reaction was stirred and allowed to exotherm on its own (no cooling). The reaction was stirred for 60 minutes (time measured from first BF<sub>3</sub> addition and BF<sub>3</sub> added over a 3–6 minute period) and then cooling water turned on. The cool reaction mixture was neutralized with 10 grams of Na<sub>2</sub>CO<sub>3</sub> and 100 ml H<sub>2</sub>O. After layer separation, the organic layer was washed twice more with fresh water and dried. The oligomer was analyzed (GPC/LC) for conversion and subjected to hydrogenation at 210° C. (2 hours), 2,000 psig H<sub>2</sub> pressure in the presence of a nickel-copper-chromium oxide catalyst (5% by weight basis weight oligomer). Stripping the oligomers of monomer was performed after hydrogenation in all of Examples 15–26 in a manner similar to that of Example 27.

##### Procedure B

Examples 19 through 23 used procedure B which was identical to Procedure A except that 0.7 g butanol was used (instead of 1.4 g) and the amount of BF<sub>3</sub> added ranged from 2.2 to 2.8 g with a 2.5 g average.

##### Procedure C

Examples 24 through 26 used Procedure C which was identical to Procedure A except that the temperature of the reaction mixture (olefin and promoter) before BF<sub>3</sub> addition was 65° C. (instead of 98° C.) and the amount of BF<sub>3</sub> added ranged from 2.2 g to 4.0 g (3.0 g average). Conversions and properties of the oligomers are summarized in Table II.

It should be noted that the amount of catalyst used in the method of this invention (1.4 to 2.8 weight percent of the olefin feed) is notably less than the amount of catalyst used in other methods in the field, such as the method disclosed in U.S. Pat. No. 4,300,006 (2.6 to 6.1 weight percent). In further contrast with the method of

this particular patent, no employment of a diluent, no heavies or lights (except monomers) removed, and a shorter reaction time are features of the inventive method. Another difference lies in the fact that the method of U.S. Pat. No. 4,300,006 uses a mixture of alpha and internal olefins having carbon numbers that are quite different from each other, unlike the instant method.

cal (being formed from the disproportionation of two alpha olefins). For example, Runs IX and XII therein oligomerize C<sub>14</sub>, C<sub>16</sub> and C<sub>18</sub> internal olefins where the double bond is at or near the center of the olefin molecule. The inventive method uses instead internal olefins where the double bond is randomly distributed instead of located near the center of a symmetrical mono olefin. These differences in the feedstocks cause important

TABLE II  
EXAMPLES ILLUSTRATING THE INVENTION

| Example | Reaction Conditions      |                          | Temp., °C. | Procedure | Con-<br>version<br>Basis LC | Properties of Hydrogenated<br>Stripped Oligomer           |       |                       |       | TGA:<br>% Sample<br>Remaining<br>at 233° C. |
|---------|--------------------------|--------------------------|------------|-----------|-----------------------------|-----------------------------------------------------------|-------|-----------------------|-------|---------------------------------------------|
|         | Feed                     | Catalyst                 |            |           |                             | Kinematic<br>Viscosity,<br>centistokes,<br>210° F. 25° C. | V1    | Pour<br>Point,<br>°F. |       |                                             |
| 15      | C <sub>13</sub> -14 int. | BF <sub>3</sub> -butanol | 98         | A         | 90.5                        | 3.82                                                      | 29.67 | 114.4                 | <-50  | 89.5                                        |
| 16      | C <sub>11</sub> -14 int. | BF <sub>3</sub> -butanol | 98         | A         |                             |                                                           |       |                       |       |                                             |
| 17      | C <sub>11</sub> -14 int. | BF <sub>3</sub> -butanol | 98         | A         | avg.                        | 4.45                                                      | 40.79 | 106.8                 | <-50  | 89.2                                        |
| 18      | C <sub>11</sub> -14 int. | BF <sub>3</sub> -butanol | 98         | A         |                             | 3.68                                                      | 29.17 | 118.1                 | -30   | 88.8                                        |
| 19      | C <sub>13</sub> -14 int. | BF <sub>3</sub> -butanol | 98         | B         | 86.4                        |                                                           |       |                       |       |                                             |
| 20      | C <sub>11</sub> -14 int. | BF <sub>3</sub> -butanol | 98         | B         |                             |                                                           |       |                       |       |                                             |
| 21      | C <sub>11</sub> -14 int. | BF <sub>3</sub> -butanol | 98         | B         | avg.                        | 4.04                                                      | 34.48 | 105.0                 | <-50  | 84.9                                        |
| 22      | C <sub>11</sub> -14 int. | BF <sub>3</sub> -butanol | 98         | B         |                             |                                                           |       |                       |       |                                             |
| 23      | C <sub>14</sub> alpha    | BF <sub>3</sub> -butanol | 98         | B         |                             | 89.1                                                      | 4.27  | 33.09                 | 134.3 | -35                                         |
| 24      | C <sub>13</sub> -14 int. | BF <sub>3</sub> -butanol | 65         | C         |                             | 83.4                                                      | 3.86  | 29.90                 | 119.4 | <-50                                        |
| 25      | C <sub>11</sub> -14 int. | BF <sub>3</sub> -butanol | 65         | C         |                             | 77.5                                                      | 5.19  | 52.54                 | 115.6 | <-50                                        |
| 26      | C <sub>14</sub> alpha    | BF <sub>3</sub> -butanol | 65         | C         | 83.6                        | 4.41                                                      | 32.70 | 148.6                 | -30   | 93.5                                        |

It may be noted from inspection of Tables I and II that alpha olefins produce invariably poorer oligomer mixtures than do internal olefins. No examples have 30 higher viscosities at both 210° F. and 25° C. than do the alpha olefin Examples 4, 8 and 11. It must be remembered that the inventive method herein has the requirement of using only internal olefins to obtain low viscosities, a feature not found in any related method. It should also be pointed out that oligomers made from alpha olefins (Examples 4, 8, 11, 23 and 26) have rather high pour points, which make them unacceptable for use in synthetic lubricants. The high pour point of Example 19 (-30° F.) is thought to be an erroneous data point.

Secondly, it may be noted that the viscosities of the BF<sub>3</sub> catalyzed oligomers are all lower than those produced by the method of U.S. Pat. No. 4,167,534. In addition, the conversions are much higher in the BF<sub>3</sub> runs. It is particularly surprising that C<sub>13</sub>-14 internal olefins (Examples 15, 19 and 24), having a higher average molecular weight than the C<sub>11</sub>-14 internal olefins (Examples 16-18, 20-22 and 25) produce olefin mixtures having a lower viscosity than the mixtures from C<sub>11</sub>-14 internals. These examples show how the choice of molecular weight range of the olefin feedstock greatly affects the properties of the product oligomers.

It is surprising that such low viscosities (relative to other methods) may be found in oligomer mixtures that also have low pour points and viscosity indexes and volatilities comparable with those of other methods. It is precisely such a blend of advantageous properties that is being sought after in the field and which has not been discovered until now.

In addition, it should be noted that the method revealed in U.S. Pat. No. 4,300,006, incorporated by reference herein, requires that the dimerization feedstock be obtained from the disproportionation of alpha olefins having 8 to 10 carbon atoms. As a result, the dimerization feedstocks therein are a mixture of alpha and internal olefins where the alpha olefins have slightly more than half the carbon number of the corresponding internal olefin and the internal olefins are highly symmetri-

35 differences in the properties of the resulting oligomers, as shown by the following examples involving C<sub>14</sub> internal olefin and C<sub>8</sub> alpha olefin as a mixed feedstock.

#### EXAMPLE 27

##### Oligomerization

The oligomerization of a 70 weight percent C<sub>14</sub> internal olefin and 30 weight percent C<sub>8</sub> alpha olefin mixture was accomplished over 2.5 g of a boron trifluoride 40 catalyst with 1.1 g of 1-butanol as a protonic promoter and initiated at 95.1° C.

To a dry and clean 300 ml Hastelloy C autoclave 45 were added 119 g of C<sub>14</sub> internal olefin from Shell Chemical Company's Higher Olefin Process (SHOP). The double bond in these internal olefins is randomly distributed throughout the molecule. Added at the same time were 51 g of C<sub>8</sub> alpha (1-octene from Aldrich Chemical Company, Inc.). At the time, this was the closest approximation possible of the U.S. Pat. No. 4,300,006 feedstock. These additions were followed by 51 1.1 g of 1-butanol promoter. The clave was sealed and the contents heated to 95.1° C. with stirring. Starting at 55 95.1° C., BF<sub>3</sub> gas was introduced by adding four shots of BF<sub>3</sub> over an 11 minute period (2.5 g total BF<sub>3</sub> added) to the stirred reaction mixture. At the end of 17 minutes (measured from the first BF<sub>3</sub> addition), the temperature had risen 110.2° C. for a maximum exotherm of 15.1° C. One hour after the first BF<sub>3</sub> addition the reaction temperature was 101.5° C. The heat was turned off and 60 cooling water turned on. The reaction mixture was neutralized with an aqueous Na<sub>2</sub>CO<sub>3</sub> solution and water washed twice more. The organic layer was separated and dried by filtering through folded filter paper to obtain a net weight of 156.3 g. Liquid chromatography analysis indicated 31.9% of the material was C<sub>8</sub>, C<sub>14</sub> or C<sub>16</sub> and 27.5% was dimer C<sub>22</sub> (from C<sub>8</sub> and C<sub>14</sub>) and 32.2% was dimer C<sub>28</sub> (from C<sub>14</sub> and C<sub>14</sub>) while 8.4% was C<sub>36</sub> or heavier. Conversion to material higher than 65

$C_{16}$  was about 68.1%. The ratio of dimer to trimer and heavies was 7.19:1.

#### Hydrogenation and Stripping

A 1-liter stirred 316 stainless steel clave was charged with 144.5 g of oligomer from the previous step and 7.2 g of a nickel-copper-chromium oxide hydrogenation catalyst. The clave was flushed with hydrogen three or four times and pressured to 1,000 psig with hydrogen. Subsequently, the clave was heated to 210° C. (the pressure increased to only 1,200 psig) and pressurized again to 2,000 psig with hydrogen. The reaction mixture was stirred at 210° C. for four hours during which the pressure remained at 2,000 psig. The hydrogenated oligomer was filtered and 137.3 g subjected to high vacuum stripping. The material was distilled through a jacketed column (with about 12 in of Goodloe packing) until the head temperature reached 105° C. at 0.06 mm Hg. The bottoms weighed 67.1 g (49.6% of the total material, overhead plus bottoms) and the overhead weighed 68.3 g (50.4% of the total material). The bottoms product had a 210° F. viscosity of 3.6 centistokes, a 25° C. viscosity of 27.4 centistokes, a pour point of < -50° F. and a viscosity index of 110. Liquid chromatography analysis indicated the presence of 25.5% dimer ( $C_{22}$ ), 60.2% dimer ( $C_{28}$ ) and 14.3% heavier materials. The TGA of the bottoms product indicated volatility was moderately high (85.0% sample remained at 233° C. in TGA of 10° C./minute).

#### EXAMPLE 28

##### Oligomerization

Oligomerization of a 70%  $C_{14}$  internal olefin-30%  $C_8$  alpha olefin mixture catalyzed by 2.2 g of  $BF_3$  with 1.1 g of 1-butanol as a promoter was initiated at 94.9° C. As in the previous example, 119 g of  $C_{14}$  internal olefin were added to a 300 ml clave along with 51 g of  $C_8$  alpha olefin followed by 1.1 g of 1-butanol. The clave was sealed and heated to 94.9° C. Starting at 94.9° C.,  $BF_3$  gas was added over an 11 minute period (totalling 2.2 g of  $BF_3$ ) to produce a 15.1° C. maximum exotherm after 16 minutes had elapsed after the first  $BF_3$  addition. After a one hour reaction time measured from the first  $BF_3$  addition, the mixture was cooled and neutralized with aqueous sodium carbonate. The organic layer was separated and dried by filtering through folded filter paper, to give a net weight of 162.5 g. Liquid chromatography analysis indicated 31.1% of the material was  $C_8$ ,  $C_{14}$  or  $C_{16}$ , 27.2% was dimer  $C_{22}$  and 33.4% was dimer  $C_{28}$  while 8.3% was  $C_{36}$  or heavier. Conversion to materials higher than  $C_{16}$  was 68.9%. The ratio of dimer to trimer and heavies was 7.30:1.

#### Hydrogenation and Stripping

From the above step, 145.0 g of the oligomer was hydrogenated over 7.2 g of nickel-copper-chromium oxide catalyst. The hydrogenation was conducted at 210° C. and 2,000 psig from hydrogen for four hours. It was followed by filtration and stripping as described in the previous example. The bottoms products amounting to 55.3% of the charge had a 25° C. viscosity of 25.7 centistokes and a 210° F. viscosity of 3.45 centistokes. The pour point of the bottoms material was unacceptably high, -40° F., and the viscosity index was 109.0. Liquid chromatography analysis indicated 33.6% dimer

$C_{22}$  and 53.8% dimer  $C_{28}$  and 12.6% heavies. The ratio of dimer to the trimer and heavies combined was thus 6.94:1. The TGA indicated 82.1% sample remaining.

#### EXAMPLE 29

##### Oligomerization

Oligomerization of a 70%  $C_{14}$  internal olefin-30%  $C_8$  alpha olefin mixture catalyzed by 2.5 g  $BF_3$  and 1.1 g 1-butanol as promoter was conducted starting at 75.1° C. To a clean and dry 300 ml clave were added 119 g of  $C_{14}$  internal olefin and 51 g of  $C_8$  alpha olefin of the same sources as the previous two examples, followed by 1.1 g of 1-butanol promoter. The clave was sealed and heated to 75.1° C. and at that temperature  $BF_3$  gas was added in increments (shots) over a 10 minute period. Five separate shots were applied to total 2.5 g. Eleven minutes after the first  $BF_3$  addition, the reaction temperature had risen to 100.7° C. (a maximum exotherm of 25.6° C.). The reaction was held at 75° C. for 1.5 hours total and then cooled and worked up as in the previous examples. The dry product from this lower temperature oligomerization had the following liquid chromatography analysis: 12.7% of monomer ( $C_8$ ,  $C_{14}$  and  $C_{16}$ ), 23.7% of  $C_{22}$ , 42.1% of  $C_{28}$  and 21.5% of trimer and heavies. Conversion to materials greater than  $C_{16}$  was 87.3% with the dimer to trimer and heavies being 3.07:1.

#### Hydrogenation and Stripping

Hydrogenation of the oligomer from the above step was completed at 210° C., 4.0 hours and 2,000 psig hydrogen pressure. Workup (filtration) followed by high vacuum stripping afforded a bottoms product which amounted to 70.7% of the charge and had the following properties: 210° F. viscosity of 4.16 centistokes, 25° C. viscosity of 34.5 centistokes, pour point of < -50° F. and a viscosity index of 124.2. The liquid chromatography analysis indicated 16.7% of the material was  $C_{22}$ , 56.8% was  $C_{28}$  and 26.5% was heavies. TGA indicated the sample had excellent volatility (90% remaining at 233° C.).

#### EXAMPLES 30-38

Examples 30-35 were conducted in a manner similar to Examples 27-29 except that certain parameters were changed as shown in Table III.

Examples 36-38 were conducted according to the following procedure. Eighty-three grams of delta 7  $C_{14}$  and 36 g of delta 9  $C_{18}$  internal olefin and 51 g of  $C_8$  alpha olefin were added to a 300 ml Hastelloy clave followed by 1.1 g of 1-butanol. This olefin mixture is the closest approximation to the U.S. Pat. No. 4,300,006 feedstocks obtainable with the materials on hand. The clave was sealed and  $BF_3$  introduced in the indicated quantities. Workup was conducted as usual involving an aqueous  $Na_2CO_3$  wash followed by two water washes and filtering the organic layer through filter paper to dry it. Hydrogenation was accomplished at 210° C. and in the presence of 5% (by weight, basis olefin) nickel catalyst and 2,000 psig hydrogen pressure for four hours. The hydrogenation product was filtered and distilled at high vacuum (<0.1 mm Hg) and to a head temperature of 110° C. The bottoms product was submitted for analysis. The results of this last set of comparative examples are summarized in Table III.

TABLE III

EXPERIMENTS USING LOWER MOLECULAR WEIGHT ALPHA  
AND HIGHER MOLECULAR WEIGHT INTERNAL OLEFINS AS FEEDSTOCKS

| Ex. | Feedstock, wt. %,                                 | Internal          | Alpha      | Reaction Temp., °C. | Reac-tion Time, Hours | BF <sub>3</sub> Added, Grams | Maximum Exotherm, °C. | Liquid Chromatography |                           | Properties of Hydrogenated Stripped Oligomers |                                         |      |                 |      |      |
|-----|---------------------------------------------------|-------------------|------------|---------------------|-----------------------|------------------------------|-----------------------|-----------------------|---------------------------|-----------------------------------------------|-----------------------------------------|------|-----------------|------|------|
|     |                                                   |                   |            |                     |                       |                              |                       | Conv.                 | Dimer, Trimer and Heavies | % Bottoms                                     | Kin. Visc., Centistokes, 210° F. 25° C. | VI   | Pour Point, °F. | TGA  |      |
| 27  | 70 C <sub>14</sub>                                | 30 C <sub>8</sub> | 95.1-110.2 | 95.1-110.2          | 1.0                   | 2.5                          | 15.1                  | 68.1                  | 7.19:1                    | 49.6                                          | 3.80                                    | 27.4 | 110.0           | <-50 | 85.0 |
| 28  | 70 C <sub>14</sub>                                | 30 C <sub>8</sub> | 94.9-110.0 | 94.9-110.0          | 1.0                   | 2.2                          | 15.1                  | 68.9                  | 7.30:1                    | 55.3                                          | 3.45                                    | 25.7 | 109.0           | -40  | 82.1 |
| 29  | 70 C <sub>14</sub>                                | 30 C <sub>8</sub> | 75.1-100.7 | 75.1-100.7          | 1.5                   | 2.5                          | 25.6                  | 87.3                  | 3.07:1                    | 70.7                                          | 4.16                                    | 34.5 | 124.2           | <-50 | 90.0 |
| 30  | 70 C <sub>14</sub>                                | 30 C <sub>8</sub> | 75.0-96.4  | 75.0-96.4           | 1.5                   | 2.5                          | 21.9                  | 93.5                  | 1.55:1                    | —                                             | —                                       | —    | —               | —    | 86.0 |
| 31  | 48.8 Δ7 C <sub>14</sub> + 21.2 Δ9 C <sub>18</sub> | 30 C <sub>8</sub> | 75.1-97.4  | 75.1-97.4           | 1.5                   | 2.1                          | 22.3                  | 83.1                  | —                         | 83.5                                          | 3.41                                    | 24.3 | 108.9           | +20  | 76.4 |
| 32  | 70 C <sub>14</sub>                                | 30 C <sub>8</sub> | 25.0-47.8  | 25.0-47.8           | 1.5                   | 2.6                          | 22.8                  | 82.0                  | 3.74:1                    | 81.9                                          | 4.91                                    | 40.8 | 138.6           | -15  | 92.9 |
| 33  | 70 C <sub>14</sub>                                | 30 C <sub>8</sub> | 25.0-28.1  | 25.0-28.1           | 6.5                   | 2.4                          | 3.1*                  | 21.4                  | 6.38:1                    | 15.5                                          | —                                       | —    | —               | —    | 83.8 |
| 34  | 70 C <sub>14</sub>                                | 30 C <sub>8</sub> | 25.0-54.5  | 25.0-54.5           | 1.5                   | 5.4                          | 29.4                  | 96.9                  | 0.93:1                    | 93.5                                          | 4.99                                    | 45.0 | 125.6           | -35  | 92.0 |
| 35  | 70 C <sub>14</sub>                                | 30 C <sub>8</sub> | 25.0-55.8  | 25.0-55.8           | 6.5                   | 5.4                          | 30.7                  | 97.3                  | 0.65:1                    | 92.8                                          | 5.91                                    | 58.4 | 126.9           | -45  | 93.6 |
| 36  | 48.8 Δ7 C <sub>14</sub> + 21.1 Δ9 C <sub>18</sub> | 30 C <sub>8</sub> | 25.2-44.4  | 25.2-44.4           | 1.5                   | 2.5                          | 19.2                  | 86.1                  | —                         | 72.0                                          | 4.40                                    | 37.1 | 120.3           | <-50 | 90.3 |
| 37  | 48.8 Δ7 C <sub>14</sub> + 21.1 Δ9 C <sub>18</sub> | 30 C <sub>8</sub> | 25.1-41.7  | 25.1-41.7           | 1.5                   | 5.1                          | 21.6                  | 93.1                  | —                         | 85.0                                          | 4.67                                    | 39.2 | 123.6           | <-50 | 90.0 |
| 38  | 48.8 Δ7 C <sub>14</sub> + 21.1 Δ9 C <sub>18</sub> | 30 C <sub>8</sub> | 25.1-51.1  | 25.1-51.1           | 6.5                   | 5.5                          | 26.0                  | 96.4                  | —                         | 85.2                                          | 5.63                                    | 54.0 | 123.2           | -40  | 94.0 |

\*This reaction never started.

35

## Conventional Base Stocks

As can be seen from Table III, the product from the feedstocks used in U.S. Pat. No. 4,300,006 are unsuitable for use as a synthetic lubricant without further distillation; i.e., the bottoms product found useful using the internal olefin feedstocks of the invention are superior. Examples 32-38 have 210° F. and/or 25° C. viscosities and/or pour points which are too high for use as 4 centistokes synthetic lubricants. These same feedstocks, when run at a higher temperature, produce a material with a low viscosity index and a poor TGA value (see Example 31).

Thus, it is determined by comparative examples using the conditions of U.S. Pat. No. 4,300,006 that the resulting products would need to be distilled in order to meet the physical properties defined for the nominal "4 centistoke fluid" of this invention, as defined previously.

## LUBRICATING OIL COMPOSITIONS

The lubricating oil compositions of this invention consist of a major amount of the synthetic lubricant component of this invention (the hydrogenated olefin oligomers described above) or a mixture of the synthetic lubricant component and a conventional base stock and minor amounts of additive components. The synthetic lubricant components used in the lubricating oil compositions hereinafter are made from olefin mixtures consisting essentially completely of internal olefins. However, it is contemplated that satisfactory lubricating oil compositions may be made from oligomers obtained from mixtures of internal and alpha olefins where the internal olefins are greater than 50 weight percent of the olefin mixture.

The conventional base stocks contemplated above, also called lubricating hydrocarbon mineral base oils, can be paraffinic base, naphthene base or mixed paraffin-naphthene base distillate or residual mineral oils, or synthesized base oils. Paraffin base distillate lubricating oil fractions are the preferred mineral oils for the formulation of crankcase lubricants. The lubricating oil base will generally have been subjected to solvent refining to improve its lubricity and viscosity-temperature relationship as well as to solvent dewaxing to remove any waxy components and to improve the pour characteristics of the oil. Suitable synthetic lubricating oils for preparing the lubricants of this invention (these are apart from the internal olefin oligomers discussed previously) include the ester base oils prepared from polyhydroxy alcohols such as pentaerythritol and trimethylolpropane and aliphatic mono-carboxylic acids, the ester base oils prepared from diacids such as dimer acid and azelaic acid and mono alkanols, synthetic hydrocarbons such as polyalpha olefins, and polyglycols and thiols, silicone fluids, polyphenyl ethers and thioethers, and the like. Generally, conventional base stocks having an SUS viscosity at 100° F. between 50 and 1,000, preferably between 70 and 500, can be used in the formulation of the lubricants of this invention. A blend of conventional base oils can be employed, if desired.

The lubricating oil compositions of this invention contain additives to enhance the performance characteristics of the synthetic lubricant component or synthetic lubricant component/conventional base stock mixture. The additives may be any of the suitable standard pour depressants, viscosity index improvers, deter-

gent-dispersants, corrosion, oxidation, and wear inhibitors, antifoamants, friction modifiers, etc. The choice of the particular additives to be included in the finished oils and the particular amounts thereof will depend on the use and the conditions desired for the finished oil product.

Specific examples of the supplementary additives are as follows:

#### Viscosity Index Improvers and Pour Depressants

A widely used and suitable viscosity index improver/pour depressant is the polymethacrylate having the general formula:



were  $\text{R}''$  is an aliphatic radical of from 1 to 20 carbons and  $n$  is an integer of between about 600 and 35,000. One of the most suitable viscosity index improvers is the dispersant polymethacrylate tetrapolymer of butyl methacrylate, dodecyl methacrylate, octadecyl methacrylate and dimethylaminoethyl methacrylate having a respective component weight ratio in the polymer of about 4:10:5:1. Another viscosity improver is a co-polymer of ethylene and propylene having a molecular weight of 20,000 to 50,000, and containing 30 to 50 weight percent propylene in the co-polymer. Another viscosity index improver is the dispersant olefin co-polymer of ethylene and propylene of 20,000 to 50,000 molecular weight containing between 30 and 50 weight percent propylene, and having pendant organo-nitrogen functionality contributing 0.1 to 0.5 weight percent nitrogen to the polymer. The viscosity index improvers and/or pour depressants are normally employed in the finished lubricant compositions in quantities between about 0.01 and 15 percent by weight.

#### Detergent-Dispersants

Examples of detergent-dispersants which can be employed are the ethoxylated inorganic phosphorus acid free, steam hydrolyzed, polyisobutene-P<sub>2</sub>S<sub>5</sub> reaction products further described in U.S. Pat. Nos. 4,272,744, 3,087,956 and 3,123,630, the adducts formed from neopentylpolyol inorganic phosphorus acid free, steam hydrolyzed polyisobutene-P<sub>2</sub>S<sub>5</sub> reaction product as further described in U.S. Pat. No. 3,281,395, the C<sub>50</sub>-C<sub>200</sub> alkenyl succinimide derivatives of alkene polyamines of the type described in U.S. Pat. Nos. 3,172,892 and 3,210,383. The succinimide derivatives are characterized by the formula:



wherein  $\text{R}'''$  is alkenyl from 50 to 2,000 carbons and  $n$  is an integer from 0 to 10. Particularly suitable examples are where  $\text{R}'''$  is polyisobutene of a molecular weight of about 1,000 to 1,500 and  $x$  is 4 or 5 and mixtures thereof. Further detergent-dispersants include the alkaline earth

metal alkylphenolates, such as barium nonylphenolate, barium dodecylcresolate, calcium dodecylphenolate and the calcium carbonate overbased calcium alkaryl sulfonates formed by blowing a mixture of calcium hydroxide and calcium alkaryl sulfonate; e.g., calcium alkylbenzene sulfonate of about 900 molecular weight with carbon dioxide to form a product having a total base number (TBN) of 50 or more, typical values being 300 to 400. Detergent-dispersants are present in the finished compositions of the invention in amounts between 0.1 and 15.0 weight percent.

#### Oxidation, Corrosion and Wear Inhibitors

Commonly employed lube oil oxidation and wear inhibitors are the divalent dialkyl dithiophosphates resulting from the neutralization of a P<sub>2</sub>S<sub>5</sub>-alcohol reaction product with a divalent metal or divalent metal oxide. Barium and zinc dialkyl dithiophosphate are specific examples. Another class of antioxidants are the polyalkylated diphenylamines, such as a mixture of 2,2'-diethyl-4,4'-diocetyl-diphenylamine and 2,2'-diethyl-4-octyl-diphenylamine. A further class of antioxidants are the polyalkylated and the polyalkylated methylene bridged phenols. Commonly employed corrosion inhibitors include the ethoxylated alkylphenol derivatives. The corrosion, oxidation and wear inhibitors are usually present in the finished lubricating oil compositions in concentrations of between about 0.01 and 3 weight percent.

#### Antifoamants

If antifoamants are employed in the finished compositions, one widely used class which is suitable are the dimethyl silicone polymers, typically employed in amounts of between about 10 and 1,000 ppm.

There are many other additives which may be useful in a lubricating oil composition as encompassed by this invention. Many of these components are listed in the disclosures of U.S. Pat. Nos. 3,864,270; 4,169,799; 4,194,981 and 4,253,980, which patents are themselves concerned with novel additives. These patent disclosures are incorporated by reference herein insofar as they teach some of the typical additives that may be useful in conjunction with the instant invention.

The following are examples of the lubricating oil compositions contemplated herein. It is preferred that the synthetic lubricant component comprise 10 to 40 weight percent of the lubricating oil composition.

#### Example 39

A SAE 5W-30 grade lubricating oil composition was derived by combining the following components:

|                  | Weight Percent                                                       |
|------------------|----------------------------------------------------------------------|
| 35.00            | Four centistoke synthetic lubricant component (described previously) |
| 0.51             | Dispersant olefin co-polymer VI improver                             |
| 0.08             | Polymethacrylate                                                     |
| 0.04             | Nitrogen as an alkenyl succinimide                                   |
| 0.24             | Calcium as an overbased calcium sulfonate                            |
| 0.12             | Zinc as a zinc dialkyldithiophosphate                                |
| 0.25             | Alkylated diphenylamine                                              |
| 0.25             | Alkylated phenol                                                     |
| 0.05             | Ethoxylated alkylphenol                                              |
| 0.50             | Friction modifier                                                    |
| 150 ppm          | Silicone polymer                                                     |
| Balance (~55.80) | Mineral oil (~300 SUS at 100° F.)                                    |

## EXAMPLE 40

A SAE 10W-30 grade lubricating oil composition was derived by combining the following components.

| Weight Percent    |                                                                                                                                                       |
|-------------------|-------------------------------------------------------------------------------------------------------------------------------------------------------|
| 33.0              | Four centistoke synthetic lubricant component (described previously)                                                                                  |
| 0.85              | Ethylene/propylene co-polymer                                                                                                                         |
| 0.40              | Polymethacrylate                                                                                                                                      |
| 0.10              | Phosphorus as neopentylpolyol adduct of inorganic phosphorus acid free, steam hydrolyzed polyisobutene-P <sub>2</sub> S <sub>5</sub> reaction product |
| 0.25              | Calcium as ovebased calcium sulfonate                                                                                                                 |
| 0.15              | Zinc as a zinc dialkyldithiophosphate                                                                                                                 |
| 0.25              | Alkylated diphenylamine                                                                                                                               |
| 0.25              | Alkylated phenol                                                                                                                                      |
| 0.35              | Friction modifier                                                                                                                                     |
| 150 ppm           | Silicone polymer                                                                                                                                      |
| Balance (~ 55.40) | Mineral oil (~ 320 SUS at 100° F.)                                                                                                                    |

The following tests were employed to demonstrate the efficiency of the lubricating oil compositions of this invention:

## Oldsmobile Sequence IID Test

The Oldsmobile Sequence IID test is detailed in "Multicylinder Test Sequence for Evaluating Automotive Engine Oils," ASTM Special Technical Publication under 315-H. This procedure is used to evaluate motor oils with respect to low temperature rusting characteristics, and was designed to relate particularly to short trip service under typical winter conditions in the upper Midwestern United States. Oldsmobile Sequence IID Test performance criteria required by the API SF Service Classification are set forth in Table IV.

## Oldsmobile Sequence IIID Test

The Oldsmobile Sequence IIID Test is detailed in the "Multicylinder Test Sequence for Evaluating Automotive Engine Oils," ASTM Special Technical Publication under 315-H. This procedure is used to evaluate the ability of motor oils to protect against high temperature oxidation, deposits and wear. The test was designed to relate particularly to high speed turnpike operation under relatively high ambient temperature conditions typical of the Southern and Southwestern part of the United States. Oldsmobile Sequence IIID Test performance criteria required by the API SF service classification are set forth in Table IV.

## Ford Sequence V-D Test

The Ford Sequence V-D Test is detailed in the "Multicylinder Test Sequence for Evaluating Automotive Engine Oils," ASTM Special Technical Publication under 315-H. This procedure is used to evaluate crankcase motor oils with respect to sludge and varnish deposits protection as well as their ability to protect against excessive valve train wear. This test was designed to simulate a combination of low speed, low temperature, "stop and go" city driving and moderate speed turnpike operation. The Ford Sequence V-D Test criteria required by the API SF Service Classification are set further in Table IV.

## CRC L-38 Test

The coordinating Research Council L-38 Test is detailed in the Federal Test Method Standard No. 791A, Method 3405.2. This test provides a method for evaluat-

ing the oxidation and copper-lead bearing corrosion characteristics of crankcase oils. The CRC L-38 Test performance criterion required by the API SF Service Classification is set forth in Table IV.

## Caterpillar 1H2 Test

The Caterpillar 1H2 Test is detailed in "Single Cylinder Engine Tests for Evaluating the Performance of Crankcase Lubricants," ASTM Special Technical Publication 509A.

This procedure is used to evaluate the effectiveness of diesel engine crankcase lubricants in inhibiting the formation of piston deposits, preventing ring sticking and preventing wear. The Caterpillar 1H2 performance criteria required by the API CC Service Classification are set forth in Table IV.

## EXAMPLE 41

The lubricating compositions given in Examples 39 and 40 were evaluated in one or more of the above-mentioned performance tests. The results are set forth in Table IV below.

TABLE IV

| Oils                                     | Example 39 | Example 40 | API SF/CC Limits |
|------------------------------------------|------------|------------|------------------|
| <u>Sequence IID Test</u>                 |            |            |                  |
| Average engine rust rating               | 8.8        | —          | 8.5 min.         |
| Lifter sticking                          | none       | —          | none             |
| <u>Sequence IIID Test</u>                |            |            |                  |
| Viscosity at 40° C. increase at 64 hr, % | 28         | 55         | 375 max.         |
| Average engine sludge                    | 9.6        | 9.6        | 9.2 min.         |
| Average piston skirt varnish             | 9.2        | 9.3        | 9.2 min.         |
| Average oil ring land deposit            | 8.0        | 7.0        | 4.8 min.         |
| Cam plus lifter wear average, inch       | 0.0021     | 0.0023     | 0.0040 max.      |
| maximum, inch                            | 0.0035     | 0.0029     | 0.0080 max.      |
| Cam or lifter scuffing                   | none       | none       | none             |
| Ring sticking                            | none       | none       | none             |
| Lifter sticking                          | none       | none       | none             |
| Oil consumption, qts.                    | 5.0        | 5.0        | 6.38 max.        |
| <u>Sequence V-D Test</u>                 |            |            |                  |
| Average engine sludge                    | 9.7        | —          | 9.4 min.         |
| Average piston skirt varnish             | 7.2        | —          | 6.7 min.         |
| Average engine varnish                   | 6.9        | —          | 6.6 min.         |
| Cam wear average, inch                   | 0.0006     | —          | 0.0010 max.      |
| maximum, inch                            | 0.0007     | —          | 0.0025 max.      |
| Oil ring clogging, %                     | 0          | —          | 10.0 max.        |
| Oil screen clogging, %                   | 0          | —          | 7.5 max.         |
| Compression ring sticking                | none       | —          | none             |
| <u>L-38 Bearing Test</u>                 |            |            |                  |
| Bearing weight loss, mg                  | 24.3       | —          | 40 max.          |
| <u>Caterpillar 1H2 Test</u>              |            |            |                  |
| Top groove fill, %                       | 15.5       | —          | 45 max.          |
| Weighted total demerits                  | 96.5       | —          | 140 max.         |

The foregoing tests demonstrate that the prescribed lubricating oil formulations prepared from the synthetic lubricant component exhibit a high level of performance in both gasoline and diesel engines, and meet the API SF/CC limits in every regard.

The oligomer mixtures produced from C<sub>13</sub>-14 internal olefins via a promoted BF<sub>3</sub> catalyst have proven to be exceptional synthetic lubricant additives. As these mixtures have a 210° F. viscosity of about four centistokes, they are considered "4 centistoke" fluids. A typical fluid of this invention was compared with the commercially available 4 centistoke decene-1 derived polyalpha-

olefin (PAO). It should be emphasized that the synthetic lubricant components of the instant invention are preferably used without further distillation after the monomer removal and hydrogenation steps. In other words, the undistilled bottoms are the finished synthetic lubricant component. The polyalpha olefins must be distilled into "2 centistoke", "4 centistoke", "6 centistoke", etc. fractions before they can be useful. Thus, the method of this invention does not require a costly distillation step, which is an important advantage over methods used by others in the field. Comparison of the properties of the fluids themselves are given in Table V. It may be seen that the fluid of this invention (A) and the commercially available four centistoke decene-1 derived PAO (B) are generally comparable.

TABLE V

| PHYSICAL PROPERTIES OF 4 CENTISTOKE FLUIDS |                   |                   |
|--------------------------------------------|-------------------|-------------------|
| TESTS                                      | A <sup>1</sup>    | B <sup>2</sup>    |
| Gravity, °API                              | 40.8              | 41.1              |
| Flash, COC, °F.                            | 430               | 435               |
| <u>Kinematic viscosity, cSt</u>            |                   |                   |
| 40° C.                                     | 17.0              | 17.1              |
| 100° C.                                    | 3.81              | 3.90              |
| Viscosity index                            | 115               | 123               |
| CCS viscosity, cP, -30° C.                 | 980               | 930               |
| <u>Brookfield viscosity, cP</u>            |                   |                   |
| -40° C.                                    | 2340              | 2200              |
| -28.9° C.                                  | 800               | 780               |
| ASTM color                                 | 0.0               | 0.0               |
| Pour, °F.                                  | <-65 <sup>3</sup> | <-65 <sup>3</sup> |
| Ash, %                                     | 0.001             | 0.001             |

<sup>1</sup>Fluid of this invention

<sup>2</sup>Commercially available 4 cSt decene-1 derived polyalpha olefin

<sup>3</sup>The actual pour points of the synthetic base oils were less than -65° F., the lowest temperature at which pour points could be measured with the equipment available.

A measure of the volatility of the two fluids is presented in Table VI where it may be seen that oligomer A is slightly more volatile than fluid B.

TABLE VI

| TEST                         | A    | B    |
|------------------------------|------|------|
| ASTM Evaporation Test        | 16.9 | 14.8 |
| % loss, 400° F./6.5 hr       |      |      |
| Thermal Gravimetric Analysis | 91   | 92   |
| % remaining at 233° C.       |      |      |
| Simulated Distillation       |      |      |
| % off column, °F.            |      |      |
| IBP                          | 687  | 619  |
| 2                            | 710  | 737  |
| 4                            | 718  | 761  |
| 6                            | 723  | 767  |
| 8                            | 727  | 771  |
| 10                           | 730  | 773  |
| 15                           | 736  | 775  |
| 20                           | 741  | 778  |
| 25                           | 745  | 785  |
| 50                           | 762  | 800  |

A lubricating oil composition was formulated from the commercially available 4 centistoke decene-1 derived PAO for comparison with the lubricating oil composition of this invention. This formulation is shown in Example 42. Except for the 4 centistoke fluid, this oil contains the same proportions of the same supplemental base oil and additives that were employed in the lubricating oil composition of Example 39. That is, the rest of the components of the two formulations are identical in type and proportion and include materials such as mineral oils, dispersants, antioxidants, detergents, friction modifiers, rust inhibitors, viscosity index improvers, pour point depressants and antifoamants. The proportion of 4 centistoke fluid (35 wt.%) is large enough

to have a profound effect on the behavior of the formulations in testing.

## 20

5 A SAE 5W-30 grade lubricating oil composition was derived by combining the following components:

| Weight Percent |                                                                                                 |
|----------------|-------------------------------------------------------------------------------------------------|
| 10             | 35.00 Four centistoke commercially available decene-1 derived PAO synthetic lubricant component |
|                | 0.51 Dispersant olefin co-polymer VI improver                                                   |
|                | 0.08 Polymethacrylate                                                                           |
|                | 0.04 Nitrogen as an alkenyl succinimide                                                         |
| 15             | 0.24 Calcium as an overbased calcium sulfonate                                                  |
|                | 0.12 Zinc as a zinc dialkyldithiophosphate                                                      |
|                | 0.25 Alkylated diphenylamine                                                                    |
|                | 0.25 Alkylated phenol                                                                           |
|                | 0.05 Ethoxylated alkylphenol                                                                    |
| 20             | 0.50 Friction modifier                                                                          |
|                | 150 ppm Silicone polymer                                                                        |
|                | Balance (~55.80) Mineral oil (~300 SUS at 100° F.)                                              |

The results of the engine tests of the two formulations are presented in Table VII. The engine tests run on the 25 two formulations are standard tests well known to those skilled in the art and have been described previously herein. It can be seen from this comparative testing that the lubricating oil composition based on the four centistoke fluid of this invention is superior to that based on the commercially available four centistoke fluid with respect to rusting characteristics as measured in the Sequence IID Test, oxidation control and oil consumption as measured in the Sequence IID Test, deposits protection as measured in the Sequence V-D Test, bearing corrosion characteristics as measured in the CRC L-38 Test, and diesel engine piston deposits protection as measured by the Caterpillar 1H2 Test. These results are further evidence of the surprisingly superior characteristics of the oligomer mixtures made from only internal olefins and a promoted BF<sub>3</sub> catalyst.

TABLE VII

| 45                        | Tests-                                   | ENGINE TEST RESULTS |            |                  |
|---------------------------|------------------------------------------|---------------------|------------|------------------|
|                           |                                          | Example 39          | Example 40 | API SF/CC Limits |
| <u>Sequence IID Test</u>  |                                          |                     |            |                  |
|                           | Average engine rust rating               | 8.8                 | 8.5        | 8.5 min.         |
|                           | Lifter sticking                          | none                | none       | none             |
| <u>Sequence IIID Test</u> |                                          |                     |            |                  |
| 50                        | Viscosity at 40° C. increase at 64 hr, % | 28                  | 242        | 375 max.         |
|                           | Average engine sludge                    | 9.6                 | 9.6        | 9.2 min.         |
|                           | Average piston skirt varnish             | 9.2                 | 9.2        | 9.2 min.         |
|                           | Average oil ring land deposit            | 8.0                 | 7.1        | 4.8 min.         |
|                           | Cam plus lifter wear average, inch       | 0.0021              | 0.0011     | 0.0040 max.      |
|                           | maximum, inch                            | 0.0035              | 0.0027     | 0.0080 max.      |
|                           | Cam or lifter scuffing                   | none                | none       | none             |
|                           | Ring sticking                            | none                | none       | none             |
|                           | Lifter sticking                          | none                | none       | none             |
|                           | Oil consumption, qts.                    | 5.0                 | 6.5        | 6.38 max.        |
| <u>Sequence V-D Test</u>  |                                          |                     |            |                  |
|                           | Average engine sludge                    | 9.7                 | 9.6        | 9.4 min.         |
|                           | Average piston skirt varnish             | 7.2                 | 6.8        | 6.7 min.         |
|                           | Average engine varnish                   | 6.9                 | 6.6        | 6.6 min.         |
|                           | Cam wear average, inch                   | 0.0006              | 0.0003     | 0.0010 max.      |
|                           | maximum, inch                            | 0.0007              | 0.0004     | 0.0025 max.      |
|                           | Oil ring clogging, %                     | 0                   | 0          | 7.5 max.         |
|                           | Oil screen clogging, %                   | 0                   | 0          | 10.0 max.        |
|                           | Compression ring sticking                | none                | none       | none             |

TABLE VII-continued

| Tests                       | ENGINE TEST RESULTS |               | API SF/CC<br>Limits |
|-----------------------------|---------------------|---------------|---------------------|
|                             | Example<br>39       | Example<br>40 |                     |
| <u>L-38 Bearing Test</u>    |                     |               |                     |
| Bearing weight loss, mg     | 24.3                | 45.9<br>39.5  | 40 max.             |
| <u>Caterpillar 1H2 Test</u> |                     |               |                     |
| Top groove fill, %          | 5.5                 | 5.0           | 45 max.             |
| Weighted total demerits     | 96.5                | 137.1         | 140 max.            |

Many modifications may be made in the method of this invention without departing from its scope which is defined only by the appended claims. For example, it would be expected that one skilled in the art could change the  $\text{BF}_3$  promoter, the temperature, pressure, modes of addition of the olefin molecular weight in trying to maximize the conversion of the oligomer properties.

We claim:

1. A lubricating oil composition comprising
  - a major portion of a synthetic lubricant component or a mixture of the synthetic lubricant component and a lubricating hydrocarbon mineral base oil, the synthetic lubricant component being made by contacting a mixture of olefins having between 9 and 24 carbon atoms, inclusive, and having greater than 50 weight percent internal olefins, where the double bond of the olefin is randomly distributed throughout the carbon chain, the balance being alpha olefins, with a catalyst comprising boron trifluoride at a temperature between about 25° and about 150° C. sufficient to effect oligomerization of said olefins, then hydrogenating the oligomerized olefins to make the synthetic lubricant component, and
  - b. minor portions of additive components.
2. The lubricating oil composition of claim 1 in which a promoter is employed in connection with the catalyst in the manufacture of the synthetic lubricant component, the promoter being selected from the group consisting of alcohols, carboxylic acids and water.
3. The lubricating oil composition of claim 2 in which the promoter is 1-butanol.
4. A lubricating oil composition comprising
  - a major portion of a synthetic lubricant component or a mixture of the synthetic lubricant component and a lubricating hydrocarbon mineral base oil, the synthetic lubricant component having a viscosity at 210° F. of between 3.5 and 4.5 centistokes, a viscosity at 25° C. of between 25 and 34 centistokes, a viscosity index of greater than 110, a thermogravimetric analysis value of greater than 86 weight percent and a pour point of less than -50° F., being produced by oligomerizing a mixture of internal olefins having between 9 and 24 carbon atoms inclusive, where the double bond of the internal olefins is randomly distributed throughout the carbon chain by means of reacting the mixture of olefins in the presence of a boron trifluoride catalyst at a temperature between 25° and 150° C. and subsequently conducting one or more mild stripping steps to remove any unreacted olefin monomer as the only separation steps, then hydrogenating the oligomerized olefins to make the synthetic lubricant component, and
  - b. minor portions of additive components.
5. The lubricating oil composition of claim 4 in which in the making of the synthetic lubricant component, the number of carbon atoms in the internal olefins of the mixture is between 11 and 14, inclusive.
6. The lubricating oil composition of claim 4 in which in the making of the synthetic lubricant component, the number of carbon atoms in the internal olefins of the mixture is 13 or 14.
7. The lubricating oil composition of claim 4 in which in the making of the synthetic lubricant component, the oligomerization is conducted in the presence of a protonic promoter selected from the group consisting of alcohols, carboxylic acids and water.
8. The lubricating oil composition of claim 7 in which the protonic promoter in the oligomerization is 1-butanol.
9. The lubricating oil composition of claim 4 in which any mild stripping is conducted at a temperature between 150° and 180° C.
10. A lubricating oil composition comprising
  - a major portion of a synthetic lubricant component or a mixture of the synthetic lubricant component and a lubricating hydrocarbon mineral base oil, the synthetic lubricant component having a viscosity between 3.5 and 5.0 centistokes at 210° F., and made by the process comprising
    - 1) oligomerizing a mixture of olefins comprising 97 weight percent or more of olefins having 13 or 14 carbon atoms and 99 weight percent or more internal olefins in which the double bond is randomly distributed throughout the carbon chain, comprising reacting the mixture of olefins in the presence of a boron trifluoride catalyst and a protonic promoter at a temperature between 25° and 150° C. sufficient to produce a crude oligomer product,
    - 2) neutralizing the crude oligomer product,
    - 3) removing the organic layer from the neutralized crude oligomer product,
    - 4) mildly stripping the unreacted olefin monomer from the organic layer of the crude oligomer product, at a temperature below 180° C., and
    - 5) hydrogenating the stripped oligomer product without further separation, and
  - b. minor portions of additive components.
11. The lubricating oil composition of claim 10 in which the viscosity of the synthetic lubricant component is about 4.0 centistokes at 210° F.
12. The lubricating oil composition of claim 10 in which in the making of the synthetic lubricant component the protonic promoter of the oligomerization step (1) is 1-butanol.
13. The lubricating oil composition of claim 10 in which in the making of the synthetic lubricant component, the mild stripping step (4) is conducted at a temperature between 160° and 180° C.
14. The lubricating oil composition of claim 10 in which in the making of the synthetic lubricant, hydrogenation step (5) is followed by a second mild stripping step to remove monomer missed in the first stripping step.
15. A lubricating oil composition comprising
  - 10 to 40 weight per cent of a synthetic lubricant component made by the process comprising
    - 1) oligomerizing a mixture of olefins having between 9 and 24 carbon atoms inclusive, the mixture being comprised of 99 weight percent or more internal olefins, where the double bond of

the internal olefin is randomly distributed throughout the carbon chain comprising reacting the mixture in the presence of a boron trifluoride catalyst and a protonic promoter at a temperature between 25° and 150° C. sufficient to produce a crude oligomer product,

- (2) neutralizing the crude oligomer product,
  - (3) removing the organic layer from the neutralized crude oligomer product,
  - (4) mildly stripping the unreacted olefin monomer from the organic layer of the crude oligomer product at a temperature below 180° C., and
  - (5) hydrogenating the stripped oligomer product, and
- b. effective portions of additive components selected from the list of components consisting of mineral oils, dispersants, antioxidants, detergents, friction modifiers, rust inhibitors, viscosity index improvers, pour point depressants, antifoamants and anti-wear agents.

16. The lubricating oil composition of claim 15 in which the internal olefins for making the synthetic lubricant component have between 11 and 14 carbon atoms, inclusive.

17. The lubricating oil composition of claim 15 in which the internal olefins for making the synthetic lubricant component have 13 or 14 carbon atoms.

18. The lubricating oil composition of claim 15 in which the promoter used to make the synthetic lubricant component is selected from the group consisting of 30 alcohols, carboxylic acids and water.

19. The lubricating oil composition of claim 18 in which the promoter is 1-butanol.

20. The lubricating oil composition of claim 15 in which the mild stripping step used to make the synthetic lubricant component is conducted at a temperature between 160° and 180° C.

20

40

21. The lubricating oil composition of claim 15 in which a second mild stripping step follows the hydrogenation step in the making of the synthetic lubricant base oil component.

22. A lubricating oil composition comprising
- a. a major portion of a synthetic lubricant component or a mixture of the synthetic lubricant component and a lubricating hydrocarbon mineral base oil, the synthetic lubricant component being made by contacting a mixture of olefins having between 9 and 24 carbon atoms, inclusive, and having 99 weight percent or more of internal olefins, where the double bond of the internal olefins is randomly distributed throughout the carbon chain, with a catalyst comprising boron trifluoride at a temperature between about 25° and about 150° C. sufficient to effect oligomerization of said olefins, separating out the unreacted olefins as the only separation step then hydrogenating the oligomerized olefins to make the synthetic lubricant component,
  - b. between 0.01 and 15.0 weight percent of a viscosity index improver,
  - c. between 0.01 and 10.0 weight percent, on an oil-free basis, of a detergent-dispersant system consisting of one or more detergents and/or one or more dispersants,
  - d. between 0.01 and 3.0 weight percent of oxidation and wear inhibitors,
  - e. between 10 and 1,000 parts per million of one or more antifoamants, and
  - f. effective portions of other additive components selected from the list consisting of friction modifiers, rust inhibitors and pour point depressants.
23. The lubricating oil composition of claim 22 in which the synthetic lubricant component is present in a proportion of between 10 and 40 weight percent.

\* \* \* \* \*

45

50

55

60

65